

March 30, 1943.

F. W. KRESSMAN

2,315,372

PROCESS OF PREPARING WOOD PRODUCTS

Filed Nov. 3, 1938

2 Sheets-Sheet 1



INVENTOR.

*Frederick W. Kressman*  
Crittton, Wiles, Davies, Nirschel & Dawson,  
ATTORNEYS.

March 30, 1943.

F. W. KRESSMAN

2,315,372

## PROCESS OF PREPARING WOOD PRODUCTS

Filed Nov. 3, 1938

2 Sheets-Sheet 2



INVENTOR.

INVENTOR.

Frederick W. Kressman,  
Chitton, Wiles, Davies,  
Kirschel and Dawson. ATTORNEYS.

## UNITED STATES PATENT OFFICE

2,315,372

## PROCESS OF PREPARING WOOD PRODUCTS

Frederick W. Kressman, Laurel, Miss., assignor  
to Continental Turpentine & Rosin Corp. Inc.,  
Laurel, Miss., a corporation of Mississippi

Application November 3, 1938, Serial No. 238,688

5 Claims. (Cl. 209—3)

This invention relates to a process of preparing a wood product, and more particularly to a process of preparing highly absorbent wood fibers of substantially uniform density.

One feature of this invention is that a process is disclosed to obtain a wood product of substantially uniform absorbent quality. Other features and advantages will be apparent from the specification and the drawings, in which:

Fig. 1 is a plan view of an air classifier; Fig. 2 is a side elevational view; Fig. 3 is an end elevation; Fig. 4 is a side elevational view, partly in section, all of the same device; and Fig. 5 is a diagrammatic view showing broadly the steps of the process of the invention.

It has long been common in the art to treat wood, such as yellow pine, to obtain therefrom turpentine, rosin and other organic products. It has been the practice to take stumps of yellow pine or other suitable wood of little value, and reduce the material to small chips by a hogging or shredding operation. The chips are steamed to remove turpentine and other volatile organic compounds, then extracted with an organic solvent to obtain the rosin, and finally steamed again to remove the solvent. After these operations, the chips have no further usefulness and are discarded or used for fuel.

I have found that these chips may be reduced to a fibrous absorbent form and in this state become adapted to many uses. For instance, the product may be used as an absorbent material in roofing felt.

Even when the wood is properly reduced to the fibrous form, extraction is desirable to provide a maximum absorbent equality. Not only are the organic liquids, which are removed, of great value, but the resulting product is much more porous. In addition, many small hard non-absorbent particles result from the fibration process. To obtain a satisfactory product, it is necessary that these be separated from the fibrous material.

I have found that wood, preferably in the form of chips or other small pieces, may be fibrated to obtain an absorbent product. At this point the wood may be extracted with a suitable organic solvent, and then treated with steam to remove the solvent. The non-absorbent particles should then be separated from the resulting product, in order to obtain a commercially useful absorbent material.

The process of fibrating the wood may be carried out in a Banbury mixer, such as that described in Patent No. 1,523,387, or other suitable machine. Although the Banbury machine was designed for

and used in the mixing of rubber, it is admirably adapted to this purpose.

In operation, the pieces of wood are subjected to frictional contact with two irregularly shaped members, which are rotated within the mixing chamber. For convenience in loading, I prefer to add to the Banbury machine an additional chamber of approximately the same size as the mixing chamber. The additional chamber may be used as a reservoir, containing a complete charge ready for introduction into the mixing chamber.

The rotating members in the mixing chamber subject the wood to frictional, twisting, shearing, shredding contact with each other and with the walls of the chamber. This action serves to reduce the wood to the fibrous form with a minimum of tearing, lacerating or breaking of the fibers. Most of the disintegration is effected along 20 the line of the grain of the wood.

In order to further reduce the laceration or breaking of the fibers, it is preferable to carry out the fibrating action in the presence of a lubricant. Most oils are suitable lubricants for 25 this purpose. However, in the fibrating of wood containing a large amount of rosin, such as yellow pine for example, the rosin in the wood acts as a lubricant. The Banbury machine, through its frictional action, develops a considerable amount of heat. The resulting temperature rise in the mixing chamber increases the effectiveness of the rosin as a lubricant.

If the temperature of the mixing chamber is controlled, it should not be maintained at less than 200—215° F. The high pressure which is developed in the process is also an aid in reducing the wood to fibrous form.

The product of the Banbury machine consists of long thin fibers of wood with smaller fibers extending therefrom, referred to herein as bundles of fibers. Most of the disintegration takes place along the lines of the grain of the wood. As a result, the fibers are of relatively small dimensions transverse to the grain. Such fibers are highly absorbent and porous, as compared to sawdust or other forms of wood reduced to small particles, such as the products of a grinding or attrition mill. To distinguish from these and other methods of reducing wood to small particles, I refer to the process of reducing wood to fibrous form by a Banbury mixer or like machine as a wood fibrating process.

The former process for recovering organic liquids from the wood, to-wit: steaming, extraction, and then steaming, when applied to the

fibrated product, tends to weaken the fibers and impair their usefulness. I have found that by treating the fibers with a volatile petroleum solvent, boiling below 250° F., substantially all of the turpentine and turpenes, as well as the rosin, may thereby be removed and recovered. Any suitable extraction apparatus may be used for this purpose. The various organic liquids removed from the wood may thereafter be separated by fractional distillation. The organic solvent may be removed from the fibers by subjecting them to steam, or, if it is not desirable to attempt to recover the solvent, merely by a conventional drying operation.

The extracted fibrated product is in a highly absorbent porous condition and contains, after the steaming operation, a high percentage of moisture usually about 40 per cent. It may be placed in a conventional dryer and the moisture content reduced to approximately 15 per cent. The step of separation of undesirable particles by means of an air classifier may be carried out with material having a moisture content as low as 1 per cent. On the other hand the same step may be carried out with material having a high moisture content although 35 per cent or more of moisture is undesirable. However, for most efficient results, I prefer to reduce the moisture only to between 12 per cent and 20 per cent.

Many of the particles found in the product are, however, relatively non-absorbent, and the product as a whole is unsatisfactory for commercial use unless these particles are removed. The absorbent qualities are not related to the size of the particles, but are directly related to their density.

By treating the fibrated product with an air classifier, substantially all of the non-absorbent particles may be removed. By the term "air classifier" is meant a device which, by passing the particles through a rapidly flowing current of air, separates them according to their densities. A specific air classifier, for example, is disclosed herein.

In an air classifier of the structure which I prefer to use, a hopper 10 is mounted above the head of a shaker table 11. From a center line peak 12 the side 13 of the table 11 is inclined downwardly to the receptacles 14 to 21, inclusive, and the side 22 is inclined downwardly to similar receptacles on the other side of the table. At the end of the table opposite the hopper 10 a V-shaped guard 23 prevents material from passing over the end of the table. Guards 24 and 25, mounted adjacent the hopper 10, serve the same purpose at the other end.

The top surface of the table 11 supports a series of riffles or fins 26 and 27 on either side of the peak. The riffles are higher at one end than the other and are mounted in such a manner that the higher ends are adjacent to the guards 24 and 25. The lower ends approach the center line of the table. Therefore, since the riffles 27 are in a position substantially parallel to each other, they are graduated in length in order that none may cross the center line of the table.

The table 11 is agitated or shaken by the eccentric 28, driven by the motor 29, and connected to the table 11 by the member 30. Resilient sliding rocker arms 31 and 32 aid in controlling the motion.

A fan 33 forces a rapidly flowing current of air through the flexible duct 34 into the chamber 35. Deflectors or louvers 36 and 37 carried by the base of the table tend to distribute the cur-

rent of air evenly along the lower surface of the table. The air then flows through a series of transverse apertures, such as the aperture 38, in the table, and through any material which may have been deposited on the table.

In operation, the fibrated extracted wood product is fed into the hopper 10 and from there deposited upon the table 11 adjacent the guards 24 and 25. The reciprocal agitation of the table 11 gradually carries the material towards the guard 23. In the meanwhile, the rapidly flowing current of air being blown through the material raises the particles of low density above the series of riffles 26 and 27 and permits them to pass down the sides 13 and 22 of the table 11 to the receptacles on either side.

The product collected in the receptacles 14 to 19, inclusive, is of substantially uniform density and of high absorbent quality, while that collected in the receptacles 20 and 21 is heavier and of lower absorbent quality. This latter material is again fed through the air classifier. The coarse material, on the other hand, passing off the end of the table, is discarded.

I have found that the highly absorbent material is also the most readily dried. Thus, when the fibrated extracted product leaves the drier, the non-absorbent particles will contain somewhat more moisture than the desired product. Since moisture increases the density of the product, this aids in the separation. Therefore, it is preferable that the average moisture content of the particles be at least 15 per cent when the particles leave the drier.

The final product consists of a wood product in the form of long, thin, porous, highly absorbent fibers from which substantially all of the organic substances, originally absorbed by the wood, have been removed. The bundles of fibers retain most of their original strength and are substantially uniform in absorbent quality. This product is extremely useful in any instance where a relatively inexpensive absorbent material is needed. For instance, this material may be used to partially or wholly replace the rag content of waterproof roofing felts.

The foregoing detailed description has been given for clearness of understanding only, and no unnecessary limitations should be understood therefrom, but the appended claims should be construed as broadly as permissible, in view of the prior art.

I claim:

1. A process of the character described for preparing highly absorbent cellulose material from wood, comprising: fibrating the wood to form fibrous particles of different absorbent quantities, the major portion of the particles being highly fibrous in character and other particles being woody and less fibrous and having a greater density than the highly fibrous particles; treating the fibrated product with moisture until moisture content of the wood is materially above 20%; heating the product to remove a portion of the moisture therefrom and reduce the moisture content of the product as a whole to between 12% and 20% whereby the differential in density between the particles is increased; and thereafter passing the partially dried product through a rapidly moving current of air to remove therefrom the particles of relatively high density.

2. A process of the character described for preparing highly absorbent cellulose material from wood, comprising fibrating the wood to

form fibrous particles of different absorbent quantities, the major portion of the particles being highly fibrous in character and other particles being woody and less fibrous and having a greater density than the highly fibrous particles, treating the fibrated product with steam to increase the moisture content to the neighborhood of 40%, drying the product in an oven to remove therefrom a substantial portion of the moisture obtained from the steam, reducing the moisture content to between 12% and 20% whereby the density differential between the particles is increased, passing the partially dried product through a rapidly moving current of air whereby the particles of relatively high density are separated from the particles of relatively low density, and collecting separately the fibrous particles of substantially uniformly low density.

3. A process for separating highly absorbent wood fibers from other particles that are woody and less fibrous into bundles of substantially uniform density comprising, treating the wood fibers with steam until the fibers contain in excess of 15% of moisture, drying the product in an oven to remove therefrom a portion of the moisture obtained from the steam, the drying operation being carried on until the fibrous product as a whole contains only approximately 15% of moisture, passing the partially dried product through a rapidly moving current of air whereby the fibers of low density are separated from the fibers of high density, and collecting separately the fibers of substantially uniformly low density.

4. A process of the character described for

5 preparing highly absorbent cellulose material from wood, comprising fibrating the wood to form fibrous particles of different absorbent quantities, the major portion of the particles being highly fibrous in character and other particles being woody and less fibrous and having a greater density than the highly fibrous particles, treating all of the fibrated particles with moisture under substantially uniform conditions to introduce a relatively large percentage of moisture into the product, subjecting all of the particles to substantially uniform drying conditions to materially reduce the moisture content of the particles whereby an increase in the density differential between the highly fibrous particles and the less fibrous woody particles is effected, and subjecting the mixture of particles to air table classification to separate the particles of low density from the particles of high density.

20 5. A process for separating highly absorbent wood fibers from other particles that are woody and less fibrous into bundles of substantially uniform density, comprising treating the wood fibers with moisture until the fibers absorb a substantial quantity thereof and containing in excess of 15% of moisture, drying the product to reduce the moisture content of the fibers as a whole to approximately 15%, and passing the partially dried product through a rapidly moving current of air whereby the bundles of fibers of relatively low density are separated from the bundles of relatively high density.

FREDERICK W. KRESSMAN.